

Feb. 16, 1937.

J. A. BECKER

2,070,644

ELECTRICAL DEVICE

Filed July 2, 1935

FIG. 1



FIG. 2



FIG. 3



INVENTOR  
J.A.BECKER

BY  
Walter C. Kiesel  
ATTORNEY

## UNITED STATES PATENT OFFICE

2,070,644

## ELECTRICAL DEVICE

Joseph A. Becker, Mountain Lakes, N. J., assignor  
to Bell Telephone Laboratories, Incorporated,  
New York, N. Y., a corporation of New York

Application July 2, 1935, Serial No. 29,441

11 Claims. (Cl. 175—366)

This invention relates to electrical devices, and more particularly to a rectifier, condenser, or the like and the method of making the same.

An object of the invention is to produce an improved electrical device of the aforementioned types.

A feature of this invention comprises an electrical device including an insulating film of one or more molecular layers thickness on a conductive or semi-conductive member or layer.

Another feature resides in the method of making such a device which comprises developing, producing or forming a film of the insulating material on a liquid and transferring the film to the conductive or semi-conductive member or layer.

Still other and further features will be apparent from the description which follows hereinafter.

In accordance with this invention, a mono-molecular film or layer of an insulating material, for instance, an oil or a fatty acid, is formed on a liquid, for instance, water, and transferred to the surface of a conductive member, for instance, a metal plate, by dipping the member in the liquid and removing it. Additional layers of the insulating material may be formed on the member by successive dippings. Subsequently, a layer of a conductive or a semi-conductive material is placed in intimate contact with the insulating layer.

A more complete understanding of the invention will be obtained from the detailed description which follows hereinafter, read with reference to the appended drawing, wherein:

Fig. 1 is a cross-section of an electrical device embodying the invention;

Fig. 2 shows a plan view of a bath in which the insulating film may be formed on a metal plate; and

Fig. 3 shows a sectional elevational view of the bath of Fig. 2 and a metal plate in various stages of treatment.

The electrical device of Fig. 1 is an electric current rectifier and comprises a disc, plate or member 10 of a conducting material, for instance, a metal, having an insulating film 11 of one or more molecular layers thickness on one surface. A layer 12 of a semi-conductor makes intimate contact with the insulating film and is engaged on its upper or outer surface by a second disc, plate or member 13 of a conducting material, such as a metal. It will be understood, of course, that the semi-conducting layer may be omitted and a device comprising the insulating film 11 between the metal plates 10, 13 be obtained.

Such a device would be a condenser. A thin film, for example, of a single or a few mono-molecular layers thickness, of an insulating material on a metal member permits the passage of current therethrough, the voltage-current characteristic being non-linear. If the film is between a pair of similar metal plates, current will flow in each direction. The capacity of this arrangement, however, is high and it is properly termed and is usable as a condenser, although having a leaking characteristic. The current passed may be decreased by increasing the thickness of the film, the latter being strictly an insulator only when thick. When a semi-conductor is inserted between the thin film and one of the plates, a greater current flows in one direction through the unit than in the reverse direction, and a rectifier is thus obtained. The insulating film is of an oil or a fatty acid that has been transferred to the member 10 by any suitable method. A preferred method will now be described with reference to Figs. 2 and 3.

The receptacle or bath 15 contains a liquid 16, for example, water, upon whose surface a film 17 of the insulating material, for instance, an oil or a fatty acid, such as stearic acid, may be initially developed as is already known by adding the insulating material to the liquid at the left of the barrier, slide or partition 18, and adjusting the position of the barrier until the layer is of a single molecular thickness. The portions 19 of the partition are out of contact with the sides of the bath, the insulating film being prevented from seeping through to the surface of the liquid to the right of the partition by the air streams 35 provided through the tubes 20.

The plate 10 at the left in Fig. 3 is shown just before it is immersed in the liquid. If it is desired merely to have a single layer of the insulating material on the plate, the latter will be 40 passed into the bath along the line A and removed from the liquid through the non-filmed surface of the bath. If it is desired to have two layers on the plate, the latter is withdrawn from the bath through the insulating film as indicated 45 by the line B. Of course, when the plate is passed through the insulating layer, the film adsorbed on the plate reduces the quantity of the insulating material and the barrier is moved to the left an amount sufficient to compensate 50 for the area of film removed, otherwise the mono-molecular layer will be destroyed. If additional layers are desired, the immersion and removal procedure is continued the necessary number of times. Subsequently, the film is removed from 55

all but one side of the plate 10 to provide the layer 11 of the device of Fig. 1. With this method of providing an insulating film on the plate 10, a film that covers the plate surface uniformly is obtained, the molecules in the film are oriented, and the number of mono-molecular layers can be accurately controlled. A test for orientation in some cases, is the action of water on the film after the plate has been removed from the bath. If the molecules are lined up on the plate with one end of the molecule in contact with the plate, water will stick to the film, while if they are lined up on the plate with the other end of each molecule in contact with the plate, water will roll off the film.

After the insulating film has been formed on the plate, a layer of semi-conducting material, such as selenium, may be vaporized thereon, and another metal placed in contact with the selenium layer or vaporized thereon. When cuprous oxide is used as the semi-conductor, it is preferable to form the insulating film on it, in the manner outlined hereinabove, and thereafter to vaporize the metal layer 10 of Fig. 1 upon the insulating film.

While this invention has been disclosed with reference to a specific device and method of manufacture thereof, it is to be understood, of course, that the scope of the invention is to be considered as limited by the appended claims, only.

What is claimed is:

1. The method of forming an insulating film on a conducting member of a rectifier, condenser or the like, which comprises developing a film of the insulating material on a liquid and transferring said film to said member.

2. The method of forming an insulating film on a conducting member of a rectifier, condenser or the like, which comprises developing a film of the insulating material on water and transferring said film to said member.

3. The method of forming an insulating film on a conducting member of a rectifier, condenser or the like, which comprises developing a film of oil on a liquid and transferring said film to said member.

4. The method of forming an insulating film on a conducting member of a rectifier, condenser or the like, which comprises developing a film of oil on water and transferring said film to said member.

5. The method of forming an insulating film on a conducting member of a rectifier, condenser or the like, which comprises developing a film of a fatty acid on a liquid and transferring said film to said member.

6. The method of forming an insulating film on a conducting member of a rectifier, condenser or the like, which comprises developing a film of stearic acid on a liquid and transferring said film to said member.

7. The method of forming an insulating film on a conducting member of a rectifier, condenser or the like, which comprises developing a film of the insulating material on a liquid and transferring said film to said member by dipping said member in said liquid.

8. An electrical device comprising a conductive member, a mono-molecular film of an insulating material formed on said member, and conductive means in intimate contact with said film.

9. An electrical device comprising a conductive metallic member, a mono-molecular film of an oil on said member, a layer of a semi-conductive material in intimate engagement with said oil layer, and a conductive member engaging with said semi-conductive layer.

10. An electrical device comprising a conductive member, a mono-molecular, oriented film of an insulating material on said member, and conductive means in intimate contact with said film.

11. The method of forming an insulating film on a member of a rectifier, condenser or the like that comprises developing a layer of the insulating material on a portion of the surface of a liquid, passing the conducting member through the layer and into the liquid, a film being thereby transferred to the conducting member, and withdrawing the member from the liquid through the portion of the surface having no insulating layer thereon.

JOSEPH A. BECKER.